

H. D. PEASE AND W. P. COHOE.  
COMPOSITE CAP OR CLOSURE.  
APPLICATION FILED AUG. 23, 1917.

1,351,438.

Patented Aug. 31, 1920.



Inventors:  
Herbert D. Page,  
Wallace P. Cohoe.  
By Their Attorneys:

Penne, Davis, Marvin & Edmonds.

# UNITED STATES PATENT OFFICE.

HERBERT DODGE PEASE, OF RICHMOND HILL, AND WALLACE PATTEN COHOE, OF RIVERDALE, NEW YORK, ASSIGNEES TO THE SANSEAL CORPORATION, OF NEW YORK, N. Y., A CORPORATION OF NEW YORK.

## COMPOSITE CAP OR CLOSURE.

1,351,438.

Specification of Letters Patent. Patented Aug. 31, 1920.

Application filed August 23, 1917. Serial No. 187,747.

*To all whom it may concern:*

Be it known that we, HERBERT DODGE PEASE, a citizen of the United States, residing at Richmond Hill, county of Queens,

5 State of New York, and WALLACE P. COHOE, a citizen of the Dominion of Canada, residing at Riverdale-on-Hudson, in the State of New York, have invented certain new and useful Improvements in Composite 10 Caps or Closures; and we do hereby declare the following to be a full, clear, and exact description of the invention, such as will enable others skilled in the art to which it appertains to make and use the same.

15 The present invention relates to closures for bottles, jars and other containers, intended primarily for containing and dispensing milk or other products, such as jams, jellies, oils, fats, mince-meat, mediacines, drugs, salts, etc. It has for its purpose to supply, in convenient form for the capping machine of a bottle or capping establishment, a disk capable of being softened by heat to a degree sufficient to permit 20 the capping mechanism to apply it securely to the open mouth of the container, whereupon, on cooling, it will set in secure and reliable sealing connection therewith.

Broadly considered, the invention comprises the employment, as the main element 30 of the material from which the disk is to be prepared, of a sheet consisting of fiber impregnated with a greater weight than itself of resinous material and mineral 35 filler, (as, for instance, filler clay). It will be convenient and preferable to supply the fibrous material of the product in the form of paper, the sheet of paper serving as a connecting web whose felted fibers will give 40 to the product the necessary flexibility and toughness. It is nevertheless intended that the resinous compound (*i. e.*, the resinous material and filler) shall be so associated with the paper in such proportion and in 45 such manner that the fibers of the paper will not, to any substantial degree, reach the exterior surface; in other words, the felted fibers of the paper will be so hermetically enclosed by and within the mass of resinous 50 compound as to be protected in their substantial entirety from the access of mois-

ture from without. In this characteristic phase of the invention, it is sharply distinguished from closures heretofore proposed, wherein the material from which the closure was made consisted of paper having a superficial coating of what was intended to be a water-resisting exterior.

In such prior closures, as far as we are aware, the effort to make the paper water-proof by impregnation with a water-proofing compound seems to have been invariably directed toward causing the water-proofing compound to subserve a subordinate rôle; that is to say, the water-proofing compound was intended and used merely as a filler, so that, in spite of whatever impregnation was effected, the fibers of the paper to a greater or less extent reached the outer surface of the completed sheet and therefore served as capillary tubes for conveying moisture to the interior. Consequently, these impregnated papers, intended to be water-proof, would not sustain for any very extended period of time 75 the demands put upon them. If submerged in water for a considerable number of hours, they will be found to have lost their water-excluding characteristics.

The underlying characteristic of the present invention, on the contrary, as above noted, consists in so combining the fibrous material with the resinous compound that the fiber will play the subordinate part rather than the compound itself. This will involve usually the employment of so relatively considerable an amount of resinous compound that, as above noted it will predominate over the weight of the paper which may even be present in so small a proportion as from 10 to 25%. Nevertheless, the presence of the paper, forming as it does a felted combination of fibers occupying the interior of the composite disks will assure the characteristics essential for 90 working or shaping the disks into the desired bottle caps or like closures and to insure that they shall take on and subsequently maintain a permanent set. The paper and the resinous compound contribute to facilitate the formation of the caps or closures and likewise contribute to their 95 100

capability for maintaining the form imparted to them by the bending and pressing operations. The presence of the mineral filler assists in making up a composite of 5 the desired toughness and tenacity, particularly when associated with the reinforcing function of the fibers.

In order to insure further the stability and resistivity of the closure, the resinous compound should be applied in such manner that 10 it will not only be present in and around the net-work of felted fibers of the paper in the predominant proportions noted, but so that it will form a surface coating which, when 15 continuous, will be practically water-resisting in the sense that it will cover substantially all of the paper fibers that might otherwise be subjected to moisture absorption, this surface coating opposing to the 20 entrance of moisture, its own full water-repelling qualities. The fiber is thus doubly protected against the prejudicial effects of moisture absorption, to wit,—the tendency 25 to cause expansion of the fibers and consequent distortion of the mass, which expansion and distortion would tend to cause the cracking of the surrounding compound with the admission of more water than would have been possible by reason of the capillary 30 conductivity of the fibers alone.

It will be understood that for some uses the supplemental outer coating of resinous compound may be restricted to but one side of the closure. On the other hand, the 35 closure may, and in many instances, will be made up of a plurality (two or more) of layers superimposed the one upon the other and united during the process of manufacture by running the layers through the compression rolls. These built up layers may 40 likewise be faced either on one side or on both sides with an outer surface or film of the resinous compound, according to the uses to which it is intended to apply the closure; 45 that is to say, whether, for such uses, it is either desirable or convenient to provide for fully protecting the closure from water penetration on one side only or on both sides.

The closure may be further supplemented, 50 (whether its main body portion consists of a single layer of fiber impregnated with the resinous compound, or of a plurality of such layers) by applying to its outer surface, either on one side or on both sides a coating 55 of non-fibrous cellulose, prepared appropriately by the viscose reaction or other preferred method. The cellulose coating thus provided has notable advantages from a practical standpoint. Thus, it is found to 60 be impervious to the resinous compound, so that the resinous compound cannot flow 65 through the cellulose with consequent surface discoloration. Further, it has the very important function of preventing the escape 70 of the characteristic odors of resin from the

resinous compound within, to such an extent that these odors are substantially imperceptible.

The non-structural cellulose coating referred to is applied to one or both sides of 70 the closure in the form of a layer prepared by the viscose reaction or the like. It effectively adapts itself to the compound-impregnated and compound-coated paper and conforms to the heating and bending operations which, in practice, are used for giving the closures their final form, and it likewise partakes of the permanent set which the closures receive as the result of their formation.

A cap or closure of this character, that is 80 to say, made up of one or more layers of fiber, combined with the resinous compound in the manner described, and having a water-resisting coating of the resinous compound and also an outer layer of non-structural cellulose is found to be capable of immersion for 85 several days in water without penetration of the water from the outer surface to the protected interior of the capped bottle or other vessel.

This result is obtained in spite of the fact that the non-structural cellulose is, of itself, not impervious to water, so that it actually presents the severe test of being water-absorbent and of presenting the water which it 95 has absorbed into very intimate contact with the underlying resinous compound, this contact being the more intimate inasmuch as the operation of applying the non-structural cellulose layer involves to some degree the 100 actual penetration of the layer into the surface of the compound.

Inasmuch as one of the important uses to which closures made in accordance with the present invention are to be put is as a 105 sanitary cap for perishable fluids, such as milk, or the like, it is desirable that the upper surface of the cap should be well adapted to the reception of a clear, sharp and durable impression by printer's ink, in order to 110 comply with the requirements of municipal authorities for a printed record on the surface of the closure of the particular day and hour of bottling. The non-structural cellulose not only presents a surface fully 115 adapted to receive a clear, sharp, and distinct print, but is found to prevent the softening up and disintegration of the fibers of the paper and the subsequent obliteration 120 or clouding of the printing which would result if the non-structural cellulose were not employed. In this respect, the printing surface presented by the closure is notably superior to the customary printing surface of the usual paper cap or closure for such 125 receptacles, wherein the action of water entering the individual filaments tends to loosen them up and disintegrate them to such an extent that the printing ink is so spread as to obscure the outlines of the 130

printed characters and render them illegible, as, for instance, when the bottles have been packed in ice for any considerable period of time.

- 5 As above noted, the non-structural cellulose layer may be applied not only to the face of the closure which is intended as the outer surface thereof, but may likewise be applied to the opposite face *i. e.*, the surface 10 next adjacent to the contents of the bottle or jar, and, in fact, the prescribed printing may be applied to said inner surface, if desired. By so doing, it would be impossible for any one to alter the printed indication of the 15 date and time of bottling, while the printed characters would be secure against obliteration, because of the superior character of the printing surface and its permanent retention thereof despite the presence of the 20 liquid contents of the receptacle. Moreover, the application of the non-structural cellulose layer to the inner face of the closure has the advantage of protecting the milk or other contents of the bottle, jar, or other 25 container from taking on the characteristic taste or odor of the resin.

A further property of the non-structural cellulose layers is that they are highly resistant to the passage of oily, fatty and 30 resinous substances, and, indeed, to all materials of a colloidal nature, and, even though absorbent to moisture, they would not tend to scuff off superficially by any ordinary accidental frictional rubbing. These are 35 qualities which correspondingly contribute not only to the permanence of the surface as a printing surface, but also to its permanence as a protection to the main body portion of the closure within.

- 40 A further advantage of the employment of the non-fibrous cellulose layers consists in the fact that in the printing operation an ink may be employed containing a dye which will unite with the non-fibrous cellulose in such a way that the printing cannot 45 be erased except by a chemical process, or by such a mechanical process as would deface the cap and therefore disclose the attempted fraud. In making up the printing 50 surface the non-structural cellulose solution employed may be given an admixture of blanc fixe, clay, or other suitable mineral substance appropriate to imparting to the coating a contrasting color to the ink employed as the printing medium.

55 While, for most uses, paper (and, in fact, paper made wholly or principally from sulfite pulp) is preferred as the material for supplying the fiber reinforcement to the 60 closure, other suitable fiber may be employed either in the form of fabric or in filamentary condition. So also, the mineral filler may be either non-fibrous or fibrous or in part fibrous and in part non-fibrous according to whether or not it is desired that

the filler shall correspondingly contribute to the reinforcing effect of the fabric fibers. These and other like modifications, within the general scope of the invention will be apparent to those skilled in the art and need not be further adverted to herein.

70 In the accompanying drawing is illustrated, in Figure 1, on a greatly enlarged scale, in section, a typical embodiment of the composite sheet from which the closures are to be cut, in the form which it assumes when made up of a series of layers, flanked on top and bottom by a layer of non-structural cellulose. Fig. 2 represents one of the closure disks. Figs. 3 and 4 represent 80 typical forms of application of the disks as closures.

In Fig. 1 of the drawing, *a* illustrates the top layer and *b* the bottom layer of viscose paper or non-structural cellulose; *c* represents the layers of paper associated with the resinous material and mineral filler and coated at *d* with resinous compound. Intermediate layers of resinous compound are indicated at *e*. Thus, for instance, in 90 building up a composite sheet, particularly adapted for supplying the disks to be used in making the closures for milk bottles and the like, in accordance with the procedure shown for instance, in United States Patent 95 to J. Bradley No. 1,160,369, it will be suitable and convenient to employ a composite sheet of the relative proportions indicated in the drawing, wherein the layers *a*, *b*, of viscose paper or non-structural cellulose 100 and the layers *c* of paper associated with resinous material and filler are of the original thickness of say .006 of an inch, the individual layers *e* of the resinous material are of, say, .009 of an inch and the coating *d* of resinous compound is of, say, .001 of an inch. The combined thickness of these layers, after compression to form the final composite sheet from which the disks are punched is ordinarily .060 to .070 of an inch. 110

115 Referring further to this drawing, the top and bottom layers *a* and *b* consist of a paper which has been impregnated with viscose carrying a mineral filler, the character of the coating and impregnation being such as to render the sheet tough and white. It presents a good printing surface and, in addition, has the property of not loosening up as to the individual fibers present when wet in water. The uncoated or pure side of these layers *a* and *b* is given a coating *e* of resinous compound carrying a mineral filler. These two sheets *a* and *b* when laid with the viscose surface outward constitute the upper and lower surfaces of the cap or 120 closure.

125 The sheets *c* constitute the main body portion of a cap or closure. As an example of one convenient method of manufacture, we may cite the following: The sheets may be 130

made by passing a sheet of paper through a coating machine which applies the resinous compound carrying the mineral filler to the sheet, impregnating it nearly, but not quite, through and through. In order to obtain a thorough impregnation, the sheet may then be coated a second time, with the result that the finished sheet which is used in making the caps or closures consists—(1) 10 of an inner portion which is made up of paper heavily impregnated with the resinous material and filler; (2) a light layer *d* of resinous material and mineral filler on the side which is coated first; and (3) a relatively heavy layer *e* of resinous material and mineral filler on the surface which was coated last.

The number of sheets which may be used to constitute the completed cap or closure will 20 vary with the purpose to which the cap or closure may be put. For instance, in some instances, a light cap consisting of four or five sheets will be employed, whereas to obtain extra mechanical strength it may, in 25 other cases, be necessary to employ 7 or 8 sheets of the gage referred to. Usually the variation in the number of sheets is not made with respect to the viscose coating sheets *a*, *b*, which constitute the outside surfaces of the finished cap or closure, but the 30 variation is made in the number of filling sheets which constitute the interior or main body portion thereof.

The sheets constituting the blank from 35 which the disks are punched, are, generally speaking, put together in one of two different ways, as follows, to wit—

1. The impregnated and coated sheets may be heated to an extent which renders 40 the compound on the surface of each sheet sufficiently warm to be sticky, and in this state the warmed sheets are passed between one or more sets of rollers, set at a proper distance apart to secure the consolidation of 45 the sheets into a composite board of the desired properties, on issuing from the pass of the rollers.

2. The consolidation may be conducted at 50 a lower temperature by using higher pressures, and, in fact, a composite sheet of greater strength may be obtained by simply warming the sheets slightly and then causing them to be acted upon between the plates of an hydraulic press, which cause 55 a consolidation and a flowing together of the adjacent surfaces of the compound.

It will, of course, be understood that the 60 illustration given in Fig. 1 of the drawing is but typical of one of the many ways in which the composite sheet or board is susceptible of embodiment. Figs. 3 and 4 illustrate typical forms of closures made from the disk shown in Fig. 2, and shown as applied to the mouth of a receptacle 65 (such as a milk bottle) *x*.

The amount of resinous compound *d*, *e*, to be employed between the individual layers *c* will depend upon the degree of waterproofing which is required when the cap or closure is used for a particular purpose. 70 For instance, if a bottle is to be capped to hold dry chemicals, it is not necessary to employ as much compound for the intervening layers *d*, *e*. In all cases, however, the amount employed should at least be 75 sufficient to cause the compound-impregnated layers of paper not only to stick together but to maintain a permanent set after the cap or closure has been applied to the bottle, jar, or other receptacle by the 80 capping machine.

It may be noted further, that the more thorough the impregnation of the paper by the resinous compound, the better are the results obtained. When, in addition to this 85 an additional layer of the compound is applied to one side of the sheet of paper already impregnated, an element of structure is presented which is almost impervious to water on the uncoated side, and practically impervious to water on the coated side. So far as we are aware, such an element or unit of structure in a closure is of itself broadly new, in addition to the structure formed by building up a number of these elements and forming therefrom a composite closure as exemplified, for instance, in the drawing. The individual units or elements making up the composite are, as hereinbefore indicated, 90 caused to adhere or stick to each other by pressure, aided by a moderate degree of heat, that is to say, a degree of heat sufficient for the purpose. It is obvious that the greater the pressure the lower is the degree 100 of heat required, and, by the employment of such high pressures as are obtainable in the hydraulic press, the consolidation of the various layers into a composite whole from which the disks, to be employed in making 105 up the caps or closures are cut may be accomplished at a comparatively low temperature. When, for instance, the individual sheets comprising the compound sheet are to be consolidated by superposing 110 them the one on the other and passing them through heated rollers, said individual sheets are led through a heated chamber, and in passing through become heated to such an extent that the resinous material becomes plastic and sticky so that when the 115 heated rollers exert their pressure upon the superposed sheets, the whole mass is melted into a composite sheet possessing the characteristic properties described.

Referring further to the non-fibrous cellulose coating, we wish to emphasize particularly its advantage in preventing the resinous compound from appearing on the outside of the cap or closure. It is found 120

that the capping operation will not force the resinous compound through the non-structural cellulose either on the upper surface of the closure so as to interfere or 5 darken the white printing surface thereof, nor will the resinous compound be forced through the inner layer of non-structural cellulose so as to stick to the bottle, jar, or the like. This prevention of the extrusion 10 of the resinous material from the heated cap is a safe-guard against its entrance into the mechanism of the crimping fingers of the machine preferred for applying the cap or closure to the receptacle, *i. e.*, a machine 15 of the Bradley type hereinbefore referred to wherein a circular series of tucking or crimping fingers, radially arranged, apply the disk to the mouth of the receptacle.

We do not restrict ourselves to the employment of non-fibrous cellulose, in so far 20 as its function is concerned of supplying a surface film or integument not soluble in water and not penetrated easily by oily or resinous materials, but may, in some instances, employ as substitutes, other substances, having these particular qualities, as 25 for instance, casein, hardened gelatin, modified starches, and the like. So also, in some instances, the inside of the cap or closure 30 may be lined with a layer of metal foil, as a protection against the action of certain corrosive liquids.

When paper is employed in the making 35 up of the composite sheet characteristic of our invention, it should preferably, as hereinbefore indicated, be formed from sulfite pulp and should have imparted to it during its passage through the paper machine a crinkled structure, by means well known 40 in the art for that purpose; so that, on issuing from the paper machine and without calendering, it may be the better adapted, by reason of its open texture and absorptive character, to readily associate itself 45 with the resinous compound and mineral filler.

What we claim is:

1. A cap or closure for bottles and other receptacles, comprising as an element of 50 structure a layer made up of a preponderating bulk of resinous compound and mineral filler associated with a reinforcement of fiber; substantially as described.

2. A cap or closure for bottles and other 55 receptacles, comprising as an element of structure a layer made up of a preponderating bulk of resinous compound and mineral filler associated with a reinforcement of fiber, said fiber being in sheet form; substantially as described.

3. A cap or closure for bottles and other 60 receptacles, comprising as an element of structure a layer made up of a preponderating bulk of resinous compound and mineral

filler associated with a reinforcement of 65 fiber, said fiber being in the form of a paper sheet; substantially as described.

4. A cap or closure for bottles and other receptacles, comprising a main body portion 70 made up of a resinous compound, a mineral filler, and reinforcing fiber, and having an outer surfacing of material insoluble in water and resistant to penetration by oily or resinous materials; substantially as described.

5. A cap or closure for bottles and other receptacles, comprising a main body portion made up of a resinous compound, a mineral 75 filler, and reinforcing fiber; and having an outer surfacing of non-structural cellulose; 80 substantially as described.

6. A cap or closure for bottles and other receptacles, comprising a main body portion made up of a resinous compound, a mineral 85 filler, and reinforcing fiber, and having on its upper surface a layer of non-structural cellulose provided with a printing surface; substantially as described.

7. A cap or closure for bottles and other receptacles, comprising a main body portion 90 made up of a resinous compound, a mineral filler, and reinforcing fiber, and having on its lower surface a layer of non-structural cellulose; substantially as described.

8. A cap or closure for bottles and other receptacles, comprising a main body portion made up of a series of individual units or elements superposed upon each other, said 100 units or elements consisting of a preponderating bulk of resinous compound and mineral filler associated with reinforcing fiber, and intervening layers of resinous compound between the said units or elements; substantially as described.

9. A cap or closure for bottles and other receptacles, comprising a main body portion made up of a series of individual units or elements superposed upon each other, said units or elements consisting of a preponderating bulk of resinous compound and mineral 110 filler associated with reinforcing fiber, and intervening layers of resinous compound between the said units or elements, and a top layer of a material insoluble in water and resistant to penetration by oily and resinous compound; substantially as described.

10. A cap or closure for bottles and other receptacles, comprising a main body portion made up of a resinous compound, a mineral 120 filler, and reinforcing fiber, and having on its lower surface a layer of non-structural cellulose and having a top layer of non-structural cellulose having a printing surface; substantially as described.

11. A cap or closure for bottles and other 125 receptacles, comprising a main body portion made up of a resinous compound, a mineral filler, and reinforcing fiber, having an upper

surfacing of material insoluble in water and  
resistant to penetration by oily or resinous  
materials, and having on its lower surface a  
layer of non-structural cellulose; substan-  
5 tially as described.

12. A cap or closure for bottles and other  
receptacles, comprising a main body portion

made up of a resinous compound, a mineral  
filler, and reinforcing fiber, and having an  
upper and lower layer of material resistant 10  
to extrusion of resin; substantially as de-  
scribed.

HERBERT DODGE PEASE.  
WALLACE PATTEN COHOE.